

# United States Patent

Fassler et al.

[15] 3,698,467

[45] Oct. 17, 1972

[54] **METHOD OF REMOVING SILACEOUS CORES FROM NICKEL AND COBALT SUPERALLOY CASTINGS**

[72] Inventors: Michael H. Fassler, Middletown; James S. Perron, Deep River, both of Conn.

[73] Assignee: United Aircraft Corporation, East Hartford, Conn.

[22] Filed: Jan. 4, 1971

[21] Appl. No.: 103,544

[52] U.S. Cl.....164/132

[51] Int. Cl. ....B22d 29/00

[58] Field of Search....164/132; 23/312 R; 134/2, 19, 134/22, 30, ; 249/61, 62

[56]

## References Cited

### UNITED STATES PATENTS

|           |         |                                |
|-----------|---------|--------------------------------|
| 3,563,711 | 2/1971  | Hammond et al. ....164/132 X   |
| 2,380,284 | 7/1945  | Young .....134/2 X             |
| 3,617,747 | 11/1971 | Wilkinson et al. ....164/132 X |

*Primary Examiner*—J. Spencer Overholser

*Assistant Examiner*—John E. Roethel

*Attorney*—Owen J. Meegan

[57]

## ABSTRACT

The removal of silaceous ceramic cores from nickel- or cobalt-based superalloy casting is effectuated by heating the casting in a solution of potassium carbonate.

3 Claims, 3 Drawing Figures



PATENTED OCT 17 1972

3,698,467



FIG. 1



FIG. 2



FIG. 3

# METHOD OF REMOVING SILACEOUS CORES FROM NICKEL AND COBALT SUPERALLOY CASTINGS

## BACKGROUND OF THE INVENTION

### 1. Field of the Invention

This invention relates to a method of removing silaceous ceramic cores from metal castings and particularly, to the removal of such cores from air cooling passages of gas turbine components which are formed of high temperature nickel- or cobalt-base superalloys. In the manufacture of metal castings, it is frequently very difficult to completely remove the silaceous material forming the core without adversely affecting the chemical composition of the surface.

### 2. Description of the Prior Art

One of the more common ways to remove silaceous core material from castings has been to immerse the part in an aqueous caustic solution or a fused salt bath. Unfortunately, such treatments tended to oxidize some of the carbides that are located in the grain boundaries and in the matrix of the alloy, thereby exposing the surface to inter- and intragranular corrosion together with a depletion of the alloy constituents along the surface. Such corrosion markedly reduced the strength of the alloys. Also disclosed have been processes embodying the use of aqueous fluoride solutions which were effective in some controlled environments for certain types of cores and alloys. But corrosion has been observed in both the nickel- and cobalt-base alloys when using this technique.

In the U.S. Pat. No. to Moir 2,502,337, a disclosure is made of subjecting a casting having a core to a treatment with fluoboric acid containing an inhibitor whereby the action of the acid on the metal can be regulated. Fluoboric acid dissolves the silica core thereby removing it from the metal casting. The process, however, can adversely affect the surface of the casting by altering its composition.

## SUMMARY OF THE INVENTION

In accordance with the present invention, the castings to be leached are immersed in an alkali metal carbonate solution at an elevated temperature, generally in excess of 200° F. The alkali metal carbonate solution is preferably saturated with the salt, but can be as low as 25 w/o. Below about 25 w/o, insufficient alkali carbonate is provided to remove the silaceous core in a reasonable time. The temperature requirements are simply that the solution and the silaceous core must be sufficiently hot to leach the silaceous material in a reasonable amount of time. We have found that the solution should be above about 200° F., preferably above boiling. Temperatures above 212° F. are realized by placing the component and the solution in a pressure vessel, commonly called an autoclave, having a heating element wrapped about the outside and arranged to raise the temperature to that which is desired. The time of the treatment is important insofar as the core is removed from the component when using the aqueous solution of alkali metal carbonate. We have found that potassium carbonate is highly desirable as the leachant because it effectively removes the silaceous material and does not adversely affect the surface of the component. Usually the silaceous material which forms the core is quartz or

fused silica and is essentially pure silica having a melting point above that of the casting.

## BRIEF DESCRIPTION OF THE DRAWINGS

FIGS. 1 to 3 of the drawings are photomicrographs taken by light metallography showing in detail the surface of superalloy castings in which cores have been removed by various solutions.

## DESCRIPTION OF THE PREFERRED EMBODIMENTS

In FIG. 1, a 500X magnification of the surface of a cobalt-base superalloy casting is shown. A core of silaceous material has been removed from the casting by dissolving it in a potassium hydroxide solution. FIG. 2 provides a 1,000X magnification of a nickel-base superalloy casting which had the core removed by potassium hydroxide also. In both cases, it can be seen that deep fissures appear on the surface of the casting. It is believed that the potassium hydroxide not only reacts with the silaceous material of the core to dissolve it, but also reacts with carbides which were disposed near the surface of the alloy. The pockets of fissures on the surface are due to the carbides washing away because of the reaction with the potassium hydroxide. In FIG. 2 there is also a depleted layer which is the result of the dissolution of alloy constituents by the leaching solution along the surface of the casting.

The rather long dark lines extending down from the surface of the casting in FIGS. 1 and 2 are corrosion lines which weaken the surface of the alloy. We have also discovered that there is no effective way of removing residual alkali material when using an alkaline hydroxide as a leachant. Some alkali is entrapped in the corroded interstices or grain boundaries and on subsequent exposure to elevated temperatures in an oxidizing atmosphere more corrosion is generated.

In FIG. 3 of the drawings, a nickel-base superalloy component which has been treated according to the process of the present invention is shown at a 500X magnification. As can be seen, neither pitting nor corrosion from the core removal treatment nor alloy depletion occurred.

As we have stated, cores from nickel- and cobalt-base superalloy castings can be removed according to the present process. Those alloys generally contain 5 to 25 w/o Cr, 5 to 15 w/o molybdenum, tantalum or tungsten, 2 to 8 w/o aluminum and titanium, less than 1 w/o carbide and the balance nickel and/or cobalt. Representative of the superalloys are those identified in the industry on the following Table I.

TABLE I

| Alloy    | Composition (% by weight)                                                            |
|----------|--------------------------------------------------------------------------------------|
| IN 100   | 10. Cr, 15. Co, 4.5 Ti, 5.5 Al, 3. Mo, 0.17 C, 0.75 V, 0.075 Zr, 0.015 B, balance Ni |
| MAR-M200 | 9. Cr, 10. Co, 2. Ti, 5. Al, 12.5 W, 0.15 C, 1. Nb, 0.05 Zr, 0.015 B, balance Ni     |
| WI-52    | 21. Cr, 1.75 Fe, 11. W, 2(Nb + Ta), 0.45 C, balance Co                               |
| MAR-M302 | 21.5 Cr, 1. Fe, 10. W, 9. Ta, 0.85 C, 0.25 Zr, balance Co                            |
| B-1900   | 8. Cr, 10. Co, 1. Ti, 6. Al, 6. Mo, 0.11 C, 4.3 Ta, 0.015 B, 0.07 Zr, balance Ni     |

The present process can also be used with nickel-base alloys such as Unimet 700, Inco 713, Inco 718 or in cobalt-base alloys such as MAR-M509, AMS-5382 and AMS-5385. The following example offers a specific embodiment of the present invention.

## EXAMPLE

300 grams of 2 were placed in a graduate and the graduate was then filled to 1,000 milliliters with water. The contents were stirred until all of the 2 was dissolved. B-1,900, a nickel-based superalloy, was placed in an autoclave which was then filled with a portion of the previously described solution. The autoclave was heated to 425° F. for 12 hours. The sample was then removed from the autoclave and washed. The silaceous material in the core had been leached and the surface was not appreciably affected.

In the following table a series of tests were performed using a 2 leaching solution. B-1,900 superalloy castings in various configurations, cast upon quarts cores, were used for the tests. The leaching rate is proportional to time, temperature, 2 concentration and the shape of the casting.

| Leaching test time | temp. | w/o K <sub>2</sub> CO <sub>3</sub> in water | Press ure in autoclave psig | Effect of K <sub>2</sub> CO <sub>3</sub> leaching on metal surface | Remarks                 |
|--------------------|-------|---------------------------------------------|-----------------------------|--------------------------------------------------------------------|-------------------------|
| 1                  | 6     | 315-345                                     | 30                          | 50-150 No Attack                                                   | Core completely leached |
| 2                  | 3     | Thermocouple broke                          | 40                          | 110-340                                                            | 85% of core removed     |
| 3                  | 6     | 430-445                                     | 40                          | 345-360                                                            | Core completely removed |
| 4                  | 6     | 345-365                                     | 30                          | 150-175                                                            | 50% of core removed     |
| 5                  | 6     | 415-445                                     | 30                          | 300-390                                                            | Core completely removed |
| 6                  | 4     | 400-440                                     | 30                          | 300-390                                                            | Core completely removed |

|    |    |         |    |         |   |                         |
|----|----|---------|----|---------|---|-------------------------|
| 7  | 5  | 400-440 | 30 | 300-390 | " | 90% of core removed     |
| 8  | 5  | 415-445 | 30 | 300-400 | " | 70% of core removed     |
| 9  | 6  | 415-445 | 30 | 300-400 | " | 80% of core removed     |
| 10 | 6  | 490-520 | 30 | 650-800 | " | 95% of core removed     |
| 11 | 6  | 490-520 | 30 | 650-800 | " | Core completely removed |
| 12 | 6  | 420-450 | 30 | 300-390 | " | 40% of core removed     |
| 13 | 12 | 420-430 | 30 | 300-380 | " | Core completely removed |

As indicated, when the core was removed from the casting there was no attack upon the surface of the alloy when using potassium carbonate solutions. The core removal is thus a function of the configuration of the casting, time, temperature, pressure, and concentration. Any of these can be modified to accomplish the removal in the shortest amount of time.

It is apparent that modifications and changes may be made within the spirit and scope of the present invention but it is our intention, however, only to be limited by the appended claims.

As our invention, we claim:

1. A method of removing silaceous cores from nickel or cobalt superalloy castings, the steps which comprise: forming an aqueous solution of alkali metal carbonate, said solution containing at least 25 weight percent alkali metal carbonate and being free of substantial quantities of caustic hydroxides; placing a nickel or cobalt superalloy casting having a silaceous core in said solution and then heating to dissolve said core from said casting.

2. The process according to claim 1 wherein said alkali carbonate is potassium carbonate.

3. The process according to claim 1 wherein said solution is heated to above its boiling point in a pressure vessel.

\* \* \* \* \*